

## UNITED STATES PATENT OFFICE

2,567,518

## PREPARATION OF BERYLLIUM NITRIDE

Alexander S. Langsdorf, Jr., Chicago, Ill., assignor  
to the United States of America as represented  
by the United States Atomic Energy Commission

No Drawing. Application June 10, 1948,  
Serial No. 32,259

5 Claims. (Cl. 23—191)

1

This invention relates to a process for the preparation of a nitride of beryllium and more particularly a process wherein beryllium nitride is prepared under controlled conditions.

An object of this invention is to provide a process for the preparation of beryllium nitride ( $Be_3N_2$ ) containing substantially the theoretical amount of nitrogen (50.8 weight percent) and having an optimum density and specific gravity. A further object of this invention is to provide a process for the preparation of beryllium nitride wherein the reaction is carried out at a controlled rate.

Other objects and advantages will become apparent to those skilled in the art upon further examination of the specification.

I have discovered that beryllium metal can be nitrided rapidly and completely by the use of hydrogen gas mixed with nitrogen in a hydrogen concentration of substantially less than 75 percent by volume. The addition of hydrogen to the nitriding system apparently exerts a catalytic action in the formation of beryllium nitride. The use of hydrogen results in increased yield over that obtained with pure nitrogen and the product formed by the process of this invention is superior to that produced by the usual nitridation processes in that the beryllium nitride formed by the process of this invention contains substantially the theoretical (about 50.8) percent by weight of nitrogen.

In accordance with the process of this invention beryllium metal is conveniently nitrided at a controlled rate by using nitrogen mixed with a controlled concentration of hydrogen. The concentration, in terms of volume percent of hydrogen present with the nitrogen, should be substantially less than 75 percent by volume of hydrogen. Up to about 50 volume percent hydrogen admixed with nitrogen is a suitable proportion since a hydrogen concentration of more than about 50 percent hydrogen reduces the reaction rate to an excessively low value. Nitrogen mixed with somewhat lower percentages, i. e. of the order of 10 percent by volume hydrogen, reacts with beryllium metal at a satisfactory rate, and an optimum rate can be achieved by using a mixture comprising between 2 and 6 volume percent of hydrogen in nitrogen.

In general the reaction time varies inversely with the temperature. The reaction takes place suitably at temperatures elevated not in excess of the melting point of the charge undergoing the reaction and proceeds at an optimum rate at

between 700° C. and 1400° C. Between these latter temperatures, the reaction is completed within about four hours. It will be apparent to those skilled in the art that the reaction time can be further substantially decreased by increasing the pressure of the gaseous reactants.

In accordance with the process of this invention, the reaction is suitably carried out in a sillimanite tube into which the nitrogen-hydrogen mixture flows in one end and the hydrogen and excess nitrogen flow from the opposite end, passing out through a throttling valve and bubbler.

In the process of this invention, it is preferred to use beryllium metal in a form such as chips to provide additional surface area for reaction with the gaseous nitrogen-hydrogen mixture.

In a further embodiment of this invention an alloy of beryllium containing a small amount, 20 i. e. about 3 percent, of an element such as aluminum, which promotes nitridation, reacts at an optimum rate with a mixture of nitrogen containing 3 percent by volume hydrogen. The beryllium nitride formed thereby contains between 47 and 49 percent by weight nitrogen and can be further reacted by reducing it to a finely-divided state, i. e. to between 40 and 60 mesh, by grinding in a beryllium mortar and pestle, pressing into pellets and refiring in the same apparatus and according to the process of this invention as previously outlined. These pellets, which have a diameter of about 1.29", swell about 0.005" on refiring. Their final density is about 1.77 and the nitrogen content approaches the theoretical value (50.8 weight percent). The pelleted product is strong, very hard, and quite stable in air. In moist air, there is slow decomposition with the expected production of ammonia; however, the product keeps well in a desiccator. The pellets are readily soluble in concentrated sodium hydroxide but dissolve somewhat more slowly in hot concentrated acid.

## Example

45

Three hundred to four hundred grams of beryllium nitride containing about 47 to 49 percent by weight nitrogen were prepared by the process of this invention in a sillimanite reaction tube measuring 1.75" inside diameter by 36" in length, 23" hot length. Beryllium chips were placed in a boat made by splitting a smaller sillimanite tube in half lengthwise. This boat was lined with a thin layer of beryllia to facilitate the removal of the reaction product. The beryllium

chips were turned from an alloy of beryllium containing 3 percent by weight aluminum. Tank nitrogen was mixed with 3 percent by volume hydrogen and passed through the reaction tube at a rate sufficient to maintain the amount of hydrogen present between 3 and 5 percent. The system was heated for about one hour until the reaction began at 870° C. and heating at about 1150° C. was continued for about four hours. Cooling from a final temperature of 1250° C. required twelve hours, bringing the total reaction time between seventeen and eighteen hours.

The nitride was then ground to 60 mesh in a mortar and pestle made from a beryllium alloy containing 3 percent aluminum and this ground nitride was then pressed into pellets in a demountable die. These pellets were then refired in contact with the gaseous nitrogen mixed with 3 percent hydrogen in the same sillimanite furnace at a temperature of about 1200 to 1300° C.

The abrasive character of the product is illustrated by the fact that on pressing pellets measuring between 1.25" by 1.50" at 60 tons pressure, about 0.0001" is worn from the die wall each time a pellet is pressed.

The process of this invention can be adapted to production on a commercial scale by using a vertical gas-tight globar heated furnace. The low density briquettes of beryllium alloy, measuring about 3.25" in diameter and about 3" high, have a hole drilled through the axis to furnish greater surface area for contact with the gaseous reactant mixture. The furnace is sealed and flushed thoroughly with nitrogen containing 3 percent hydrogen until the reaction rate is increased sufficiently to maintain the reaction without further appreciable electric heating.

From about 12 lbs. of the briquettes made from the beryllium-aluminum alloy, about 23 lbs. of beryllium nitride containing at least about 46 percent by weight nitrogen are produced within 18 hours. This beryllium nitride is crushed in a power-operated jaw-crusher to a size sufficient to pass a 40- to 60-mesh screen and is formed into pellets having a specific gravity of about 1.7 and subjected to further nitriding at about 1300° C. in the globar furnace. The beryllium nitride pellets increased both in dimensions and density relative to the amount of additional nitrogen taken up on refiring in the nitriding operation, so the process must therefore be carefully controlled if the pellets are to be used in cans of

a predetermined size. Obviously the change in size on refiring will be less if, prior to refiring, the nitride material contains close to the theoretical weight of nitrogen.

The foregoing descriptions comprise the preferred embodiments of this invention. However, many alterations and changes may be made therein without departing from the spirit and scope of this invention as set forth in the appended claims which are intended to cover, as broadly as possible in view of the prior art, all features of novelty, either singly and/or in combination.

What is claimed is:

15. 1. A process for the preparation of beryllium nitride comprising heating beryllium metal in contact with a mixture consisting of nitrogen and hydrogen wherein the concentration of hydrogen is between 2 and 6 percent by volume hydrogen.
20. 2. The process of claim 1 wherein the temperature of the reaction is between 700 and 1400° C.
25. 3. The process of claim 2 wherein the metal reactant is in a fine state of sub-division.
30. 4. A process for the preparation of beryllium nitride containing nitrogen in an amount substantially identical with the amount of nitrogen present in the compound of the formula  $Be_2N_2$  and having an increased density, comprising pressing a pulverized and partially nitrided beryllium into pellets and refiring said pelleted and nitrided beryllium at 1200 to 1300° C. in contact with nitrogen containing about 2 to 6 percent by volume hydrogen.
35. 5. A process for the preparation of beryllium nitride comprising heating a beryllium alloy consisting of beryllium and about 3 percent by weight aluminum at a temperature of about 1200° C. with a binary gaseous mixture consisting of nitrogen and between 2 and 6 percent by volume hydrogen gas.

ALEXANDER S. LANGSDORF, JR.

#### REFERENCES CITED

45. The following references are of record in the file of this patent:
  - Fichter et al., Zeitschrift fur anorganische und allgemeine Chemie, vol. 93, page 88 (1915).
  - Satoh, Nature, vol. 133, page 837 (1934).
  - 50. Mellor, Comprehensive Treatise on Inorganic and Theoretical Chemistry, vol. 8, page 153 (1928).